

## UNITED STATES PATENT OFFICE

2,131,138

## TREATED LUBRICANT

Albert Ernst Ganzert, Chicago, Ill., assignor to  
Ernest C. ShawNo Drawing. Application December 11, 1935,  
Serial No. 53,999

4 Claims. (Cl. 87—9)

This invention relates to a treated lubricant, and to a method of treatment for improving the qualities of lubricants subjected thereto.

One object of this invention is to produce a finished lubricant which will form a highly persistent and tenacious lubricating film on a surface; another object is to produce a film forming lubricant whose film remains substantially intact when exposed to the action of water, water vapor, the wiping action of rolling or sliding parts, the scrubbing action of foreign material, the displacing action of heat and load, and the dissolving action of solvents derived from hydrocarbons, such as gasoline, kerosene, etc. Yet another object of this invention is to provide a finished lubricant having a high degree of oiliness and penetration and resulting in a lower coefficient of friction between surfaces, while at the same time forming a film which persistently adheres to such surfaces; other and further objects and advantages will appear in the specifications following.

I have found that by treating an ordinary refined hydrocarbon lubricant with fatty acid salts of polyvalent bases, particularly of aluminum, and mono or dibasic oxides and their like fatty acid salts, as zinc for example, in proper proportions, a change is produced in the lubricant giving it the qualities or characteristics mentioned above, along with other desirable qualities.

I have found that, generally speaking, the higher the molecular weight of the fluid or substance being used as a lubricant, the lower the coefficient of friction between two surfaces separated by a film of such substances. For example, the coefficient of friction between two pieces of polished hard steel having a film of hydrocarbon lubricant known as undecane between them, which particular lubricant has a molecular weight of 156, is .517. Where a hydrocarbon lubricant having a higher molecular weight is used, such as tetracosane having a molecular weight of 338, the value of the coefficient of friction between the steel surfaces is reduced to .165. Assuming the lubricants to be composed of saturated hydrocarbons, it can be seen that the reduction in the coefficient for each  $\text{CH}_2$  group added is considerable, the reduction from undecane (about the lowest molecular weight suitable for general lubricants) to tetracosane being about 68%. The difficulty with the saturated hydrocarbons of higher molecular weight, however, is that they produce a fluid which is unsuitable for ordinary lubricant use, since it is either exceedingly viscous or even solid at normal temperatures.

Tetracosane, for example, is solid at ordinary room temperature and only a very small percentage can be present in a fluid lubricant without destroying its possibilities for ordinary commercial uses.

The reduction in the coefficient of friction as molecular weight increases is also found in connection with other substances than pure hydrocarbons. Certain acids, for example, having lubrication properties which result in low coefficients of friction between adjacent metal surfaces. Stearic acid, for example, having a molecular weight of 284 produces a coefficient of friction under the above conditions of .0052.

It is clearly deducible from these results that if still larger molecules could be used and could be kept in a fluid state at low temperatures, great benefit would accrue to the lubricants from their presence. In order to obtain the benefit of such higher molecular values I have made use of fatty acid salts of polyvalent bases in the usual refined hydrocarbon lubricant. As an instance of my invention, I will take as a specific example, aluminum stearate having a molecular weight of 877, which is three and one-half times that of octadecane, the highest molecular weight saturated hydrocarbon which remains liquid at normal temperatures. I have found, however, that even when small quantities of aluminum stearate are dissolved in a hydrocarbon lubricant it adds to the oil excessive and undesirable viscosity. Such a product, without further treatment, is impractical for ordinary lubrication purposes, as in an automobile engine.

I have found that the addition to such a product, of reagents of a precipitating character, such as zinc oxide along with a like fatty acid salt of the same base (zinc stearate in this case) in certain definite proportions, results in a reduction of the viscosity of a plain solution of aluminum stearate, substantially lowering the viscosity of this final mixture below that of the plain untreated hydrocarbon lubricant in the cold and maintaining a slightly higher viscosity at elevated temperatures. It is necessary to add these reagents in quantities just short of the precipitating amounts, so that the resulting compound takes on the character of a colloid or colloidal suspension wherein the heavier molecules are dispersed throughout the hydrocarbon medium and remain suspended therein.

The following is given as an example to illustrate the changes in viscosity produced by the addition of the zinc salts. A commercial straight mineral oil having a S. A. E. viscosity rating of 55

40 was used as a base, and in it was dissolved by heating, at about 200° F., 1.782% by weight of aluminum stearate, a monobasic fatty acid salt of aluminum. A mixture of zinc stearate and zinc oxide was then made up, the compound containing approximately 15% zinc oxide. This compound was then added to another similar solution (S. A. E. 40 mineral oil and 1.782% aluminum stearate) in just sufficient quantities so that no 10 floc was formed when the resulting compound was dissolved in a light benzine. For comparison, the two treated lubricants will be called Nos. 1 and 2, No. 1 being the hydrocarbon and 1.782% aluminum stearate, No. 2 being the same as No. 1 plus the zinc salts. The Saybolt viscosities gave 15 the following results:

|    | No. 1       |                 | No. 2       |                 |
|----|-------------|-----------------|-------------|-----------------|
|    | Temperature | Saybolt seconds | Temperature | Saybolt seconds |
| 20 | Degrees F.  |                 | Degrees F.  |                 |
|    | 240         | 252             | 240         | 56              |
| 25 | 210         | 390             | 210         | 74              |
|    | 130         | (*)             | 130         | 368             |
|    |             |                 | 100         | 889             |

\*Impossible to take.

Not only does the lubricant No. 1 have more 30 than five times the viscosity at 210° F., as does lubricant No. 2, but lubricant No. 2 also shows greater resistance to displacement by heat, water, water vapor, pressure, the wiping action of rolling or sliding parts and the scrubbing action of foreign materials but also shows a lower coefficient of friction. From .5 to .67% of the compound as in No. 2 above is sufficient to give very beneficial results to the untreated oil.

Although zinc oxide is a precipitant for aluminum salts, the reaction between zinc oxide and aluminum stearate or other monobasic fatty acid salt of aluminum is such that it requires three molecules of zinc oxide to precipitate two molecules of aluminum stearate. In the making of the 45 compound, above identified as No. 2, approximately five molecules of the aluminum salt to one molecule of zinc oxide was used. Slight or partial precipitation from a molecular solution, as here, forms aggregates within the colloidal size 50 range. In order to maintain this state of equilibrium, it is necessary that each separate particle somehow be prevented from gathering with other similar particles to form larger aggregates which would precipitate. It has been found that 55 in the fabrication of the complex compound or finished treated lubricant, identified as No. 2, small changes from the critical proportions will cause flocculation and subsequent precipitation.

It is believed that the above proportions of 60 zinc salts and aluminum stearate are just sufficient to cause a rearrangement of the electron systems within the molecule, thus developing an electrical charge on each particle which repels other like particles and enables them to maintain 65 a separate existence. This same charged particle, moreover, is attracted to, and firmly held upon, any surface exhibiting an opposite charge, to the full neutralization of that opposite charge. It is believed that this is the reason 70 for the adsorbed film which clings to the metal surfaces. It also follows that any rupture of this adsorbed film will be instantly replaced so long as properly charged particles remain in the lubricant medium flowing across the metal surface.

75 Whether or not this be the true explanation,

however, it is a fact that oil treated, as disclosed herein forms a film of adsorbed molecules on the metal surface of a bearing or the like, which film clings much more tenaciously than is the usual case and repairs itself more quickly if ruptured 5 for any reason.

Metals, particularly iron, seem to possess an attractive field of force, electromagnetic in character, near their surfaces. This force, similar to the better known term cohesion, holds two 10 adjacent metal surfaces together and is one of the principal causes of friction. It therefore follows that the thicker the film of lubricant between the surfaces, the less the attractive force between the same surfaces, since the factor of 15 distance diminishes such force rapidly. Considering again this adsorbed film, it is clear that the larger the size or volume of the molecules of which it is construed, the greater the distance between the rubbing surfaces will be, and, if this 20 adsorbed film is composed of substances that will resist the compressive effect of pressures or load to a greater degree than ordinary hydrocarbon, the film will continue to function under conditions that would otherwise cause failure. 25

In order to increase the adsorbing ability of the lubricant film and thus to add to the load carrying ability of the above-mentioned lubricant, it has been found advantageous to add a small percentage of some chlorine derivative of 30 the hydrocarbons, especially the lower hydrocarbons. These chlorine derivatives are preferably of the class in which all of the hydrogen atoms are replaced by chlorine atoms, as for instance carbon tetrachloride. For example, a 35 straight paraffin oil having an S. A. E. viscosity of 30 was used for a test, and to one sample thereof one per cent of the above-mentioned aluminum zinc compound was added and a little over 3% of carbon tetrachloride. The straight 40 oil, tested on a film strength testing machine, seized at 7,500 pounds per square inch. The treated sample of the same oil was run on the same machine to 73,500 pounds per square inch, which was the limit of the capacity of the machine, and no seizure occurred. In addition, such treated oil suffers much less change in color under heating in an oven for twelve hours at 350° F., and shows no corrosive effects, whatsoever, on pieces of metal and bearing alloys 50 immersed in the oil for nine hours at about 300° F.

For illustrative purposes in the foregoing example, carbon tetrachloride was mentioned. In practice all of the halogen derivatives of the 55 lower hydrocarbons seemed to be advantageous, and the particular halogen derivative suited to the conditions under which the lubricant will be required to function would be chosen. Where heat of combustion is practically absent, carbon 60 tetrachloride would be used on account of its relatively low cost since carbon tetrachloride has a boiling point around 170° F. However, carbon dichloride would be used where the oil temperature of the bearing surfaces would be around 65 200° F., for example. Where both load and combustion heat are higher carbon trichloride would preferably be used, since this has a boiling point of about 365° F. Where available and cost considerations do not interfere with its use bromine 70 (having an atomic weight of 79.92 as against that of chlorine, 35.46) may be substituted for chlorine where it is desired to operate under higher temperatures.

The foregoing detailed description has been 75

given for clearness of understanding only, and no unnecessary limitations should be understood therefrom, but the appended claims should be construed as broadly as permissible, in view of 5 the prior art.

What I claim as new, and desire to secure by Letters Patent, is:

1. A lubricant of the character described, having a low coefficient of friction and adapted to 10 form a persistent film stable under high temperatures and pressures, including; a hydrocarbon adapted to be used as a liquid lubricant; from three-tenths to five per cent of aluminum stearate; and less than one-twenty-fifth as much 15 zinc oxide and less than one-fifth as much zinc stearate.

2. A lubricant of the character described, liquid at ordinary temperatures, having a low coefficient of friction and adapted to form a persistent film stable under high pressures and tem- 20

peratures including: a hydrocarbon oil; a small proportion of aluminum stearate; a quantity of a mixture of zinc stearate and zinc oxide large enough to cause colloidal suspension of the compounds of metals present in said lubricant and 5 small enough that precipitation of said compounds will not occur.

3. A lubricant of the character described, liquid at ordinary temperatures, having a low coefficient of friction and adapted to form a persistent film stable under high pressures and temperatures including: a hydrocarbon oil; approximately 2.5% of aluminum stearate; approximately 0.1% of zinc oxide; and approximately 10 15 0.6% of zinc stearate.

4. A lubricant of the character described in claim 1 including less than 5% of carbon tetrachloride.

ALBERT ERNST GANZERT. 20